

## UNITED STATES PATENT OFFICE

2,362,289

## LUBRICATING COMPOSITIONS

Louis A. Mikeska, Westfield, N. J., assignor to  
Standard Oil Development Company, a corporation of Delaware

No Drawing. Application December 16, 1938,  
Serial No. 246,073

24 Claims. (Cl. 252—48)

This invention relates to improved oxidation inhibitors which are particularly effective in mineral oils and lubricating compositions, particularly to metal derivatives of phenol sulfides.

It has been found that both the stability and lubricating properties of hydrocarbon oils are improved by adding thereto small amounts of metal derivatives of phenol sulfides. These compounds include metal salts of phenol sulfides which are represented by the following formula: 10



in which M represents a metal, such as aluminum, barium, calcium, cobalt, chromium, magnesium, manganese, sodium, nickel, lead, tin, zinc, copper, iron, cadmium, potassium, lithium and the like. In the case of polyvalent metals, other valences than that connected to the oxygen in this formula may be joined to other inorganic or organic groups, such as halogen, sulfur, oxygen, alkyl and aryl groups, residues of alcohols, phenolic compounds, mercaptans, organic and inorganic acids, such as —OR'' and —SR'', and the like, in which R'' represents an organic or inorganic group or radical. R' represents an organic group which may be either aryl, alkyl, aralkyl, or alkyl-aryl and which may contain substituent groups, such as halogen, particularly chlorine, also nitro, nitroso, amino, hydroxy, carboxy, alkoxy, aroxy, mercapto, and the like. R represents an organic group of the same class as R', and which may also contain the same substituent groups, but is preferably an alkyl group of about 4 to 8 carbon atoms.

The hexagon represents an aromatic nucleus containing 1 or more benzene rings or a condensed ring system, such as in naphthalene and the like. The hexagon may also contain any one or more of the substituent groups described in connection with the group R'.

The positions of the various groups attached to the hexagon are not limited to those shown above, this formula being merely illustrative, but may also be in any other ortho, meta, or para relation to each other.

The sulfur atom represented by S in the above formula may be substituted by selenium or tellurium. The subscript x represents an integer between 1 and about 5 and is preferably 1 or 2.

Metal salts of alkyl phenol sulfides and polymers thereof have been found particularly effective improving agents for lubricating oils. These alkyl phenol sulfides include the following classes:

## 1. Alkyl phenol thioethers



## 2. Alkyl phenol disulfides



and



## 3. Polymers of alkyl phenol sulfides



and



## 4.



## 40

While the above compounds are preferably symmetrical, one or more of the benzene nuclei may contain other substituent groups, such as represented by the following formula:



## 5. Dinitro phenyl alkyl phenol sulfide

In all the above Formulae 1 to 5, R represents an alkyl group containing preferably about 4 to 8 carbon atoms.

This invention relates to metal derivatives of all such compounds, in which the hydrogen of one or more of the hydroxyl groups is replaced by a suitable metal such as those described above. In the case of polyvalent metals, the metal may be connected to two hydroxyl groups of the same molecule or it may join two different

molecules, which may be similar or different, at least one of the molecules being a phenol sulfide. Illustrative salts are represented by the following formulae:

7.



8.



9.



The groups R, S<sub>2</sub>, R' and R'' in the above formulae are the same as those described above. OR'' is preferably the same group as the other organic group attached to the nickel.

Illustrative compounds and suitable methods for their preparation are as follows:

#### EXAMPLE I

1 mole of tertiary amyl phenol thioether (prepared by the method described in the French Patent 824,600) is dissolved in about 1½ times its volume of absolute ethyl alcohol. This solution is then added to a solution of sodium ethoxide, prepared by dissolving 2 moles of metallic sodium in an excess of absolute ethyl alcohol. The sodium salt of the phenol, described as the thioether of tertiary amyl sodium phenolate, is thereby formed and remains in solution in the excess ethyl alcohol.

It may be recovered by evaporation of the alcohol, or the solution may be added directly to a lubricating oil, in which case the alcohol may be removed by evaporation in case a lubricant having a high flash point is desired.

Other metal salts may be prepared from the sodium salt by a simple double decomposition reaction which is illustrated in the following example:

#### EXAMPLE II

A slight excess over the calculated amount of the anhydrous halide (chloride or bromide) of the desired metal, such as calcium chloride, is dissolved in absolute ethyl alcohol, and the resulting solution is added with stirring to the alcoholic solution of the thioether of tertiary amyl sodium phenolate described in the preceding example. The thioether of tertiary amyl calcium phenolate (calcium salt of dialkyl dihydroxy diphenyl sulfide) is thus formed along with sodium chloride, which is insoluble in the absolute alcohol and precipitates therefrom. The mixture is then filtered to remove the precipitated sodium chloride and the alcohol removed by evaporation of the filtrate, the last stage of the evaporation being conducted under vacuum. If it is found that the sodium chloride is not completely removed, due to the presence of traces of water or other reason, the product may be further treated to remove the sodium chloride by any suitable means. For example, the dried product may be dissolved in petroleum naphtha in the

absence of water. The sodium chloride remains undissolved and is separated from the naphtha solution by filtration.

The above procedure may also be used in preparing corresponding thioether phenol salts of aluminum, magnesium, zinc, barium, and cobalt. The chlorides of the metals are satisfactory in all cases except with barium, in which case it is preferable to use the bromide in order to secure sufficient solubility of the barium halide in absolute alcohol.

In some cases it will be found that some of the metal salt of the phenol thioether precipitates along with the sodium chloride. It may be recovered by extracting the dried precipitate with 54 Bé. naphtha. The desired product is then obtained in concentrated form by evaporation of the naphtha.

Absolute methyl alcohol may also be used as solvent in place of the ethyl alcohol in the same processes described above. It is preferable to use methyl alcohol as a solvent in the preparation of the corresponding nickel salts of phenol thioethers, as nickel chloride is only slightly soluble in ethyl alcohol.

#### EXAMPLE III

Thioether phenolates of metals having sufficiently basic oxides may be prepared by a direct reaction of the phenol thioether and the oxide in the following manner: A mixture of 107 parts of tertiary amyl phenol thioether, 214 parts of xylol, 10.8 parts of water, and 16.8 parts of hydrated calcium oxide was heated to boiling under a reflux condenser provided with a trap for removing water from the reflux condensate. The refluxing was continued until all the water (16.5 parts) had been removed. There was thus obtained an xylol solution of the thioether of tertiary amyl calcium phenolate (calcium salt of dialkyl dihydroxy diphenyl sulfide). The excess calcium oxide (or hydroxide) was insoluble in the xylol and was removed by filtration. The calcium salt of the tertiary amyl phenol thioether was then obtained by evaporation of the xylol from the filtrate.

This process may also be conducted with other basic oxides or hydroxides, such as those of barium, sodium, potassium etc.

#### EXAMPLE IV

Metallic magnesium was converted into the alcoholate by stirring with an excess of absolute ethyl alcohol in the presence of mercury chloride and iodine as catalysts. A solution of tertiary amyl phenol thioether in absolute ethyl alcohol was then added to the resulting suspension of magnesium ethoxide. The mixture was refluxed for 24 hours and was then filtered while hot to separate insoluble material. The filtrate was then evaporated to dryness and there was recovered as residue the thioether of tertiary amyl magnesium phenolate.

#### EXAMPLE V

One part of anhydrous sodium hydroxide is suspended in 3 parts of 98% strength isopropyl alcohol. The theoretical amount of tertiary amyl phenol thioether for neutralization of the phenolic hydroxyl groups by the sodium hydroxide was then added. The resulting solution was then heated to boiling and two parts of the alcohol were distilled off. This rendered the distillation residue substantially anhydrous, since the distillate isopropyl alcohol is of 91% strength

so long as water is present in the mixture being distilled. There was thus obtained a solution of the thioether of tertiary amyl sodium phenolate in absolute isopropyl alcohol.

Salts of other metals may be prepared by using the halides of such metals as described in Example II. For example, the theoretical amount of anhydrous calcium chloride is added to the distillation residue and the suspension heated under reflux until the calcium chloride has all reacted. The precipitated sodium chloride is then removed by filtration and the thioether of tertiary amyl calcium phenolate is obtained as a residue by evaporation of the isopropyl alcohol. Other metal halides may be used in place of the calcium chloride, for example, barium bromide, lithium chloride, or any other metal halide which is soluble in dry isopropyl alcohol.

#### EXAMPLE VI

100 parts of benzene are added to 100 parts of 95% alcohol containing 25 parts of tertiary amyl phenol thioether and enough sodium hydroxide to neutralize the latter. The resulting solution is heated to boiling and water removed in the constant boiling mixture benzene-water-alcohol which distills over. Thereafter anhydrous calcium chloride is added to the distillation residue, which is an anhydrous solution in benzene and alcohol and the reaction is completed in the same manner as in Example V.

A solution of calcium chloride in 95% ethyl alcohol may be used, instead of anhydrous calcium chloride, in which case the water present in the alcohol is removed by further azeotropic distillation. After removal of the water, the preparation of the thioether of tertiary amyl calcium phenolate is completed as described in Example V.

Corresponding metal salts of alkyl phenol disulfides and polysulfides and of the polymers, such as the dimers, trimers, and tetramers of the alkyl phenol thioethers, disulfides, and polysulfides, may also be prepared by substituting the respective alkyl phenol sulfide for the alkyl phenol thioethers used in the above examples. Metal salts of the corresponding selenides and tellurides may also be prepared by similar methods.

The crude products may also, if desired, be subjected to further purification in addition to, or in combination with or in place of the distillations described above. Preparation of products of enhanced purity may be accomplished by fractional crystallization, by extraction or precipitation with selective solvents. Impurities may also be removed by treatment with suitable adsorptive agents, such as clay.

While these compounds, or mixtures thereof with other members of the same class and with the corresponding alkyl phenol sulfides, may be added in any desired concentration within their solubility limits to lubricating oils, they are preferably used in concentrations of about 0.01 to 2.0%; a concentration of about 0.05 or 0.1 to 0.25% will be found sufficient to stabilize the majority of petroleum lubricating oils. Larger proportions of about 5% or more may be used to improve the lubricating properties of the oil.

The compounds described above may be used as oxidation inhibitors and improving agents in similar concentrations in other hydrocarbons, such as waxes, fuel oils, Diesel oils, naphthas, burning oil, gasoline, and the like.

These compounds may also be used as oxida-

tion inhibitors generally in organic materials which are subject to degradation by oxidation during normal conditions of storage or use, or which tend to deteriorate by absorption of oxygen from the air. Illustrations of such materials are: fatty oils, petroleum oils and their derivatives, soaps, aldehydes, synthetic resins, rubber, synthetic rubber, paper and the like.

These compounds greatly improve mineral lubricating oils including the highly refined oils such as synthetic oils, solvent extracted oils obtained by treatment of mineral lubricating oils with single solvents such as phenol, dichlorethyl ether, furfural, propane, nitrobenzene, croton-aldehyde, etc., or by double or multiple solvents such as propane-cresol, etc., clay or acid treated oils, also aluminum chloride treated oils, white oils, hydrogenated oils, and the like. The lubricating oils improved by these compounds also include light mineral oils such as spindle oils and oils used generally for textile treating, metal cutting oils, turbine oils, insulating and transformer oils, automobile and Diesel crankcase lubricants, steam cylinder oils, and greases. The oils to which these improving agents are added may be either in the crude form or partially or highly refined by distillation, volatilization, chemical reagents, and adsorptive agents; as well as coal tar or shale distillates, pale oils, neutrals, bright stocks and other residual stocks, cracking coil tar fractions, condensed or polymerized fractions, and the like, either waxy, dewaxed, or non-waxy. They are especially desirable for addition to crankcase lubricants used in internal combustion engines and to other lubricants which are used at elevated temperatures above about 150 to 200° C.

The lubricants and other oxidizable organic materials to which these improving agents are added may also contain dyes, metallic or other soaps, pour inhibitors, sludge dispersers, oxidation inhibitors, thickeners, V. I. improvers such as soluble linear polymers, oiliness agents, resins, rubber, fatty oils, heat thickened fatty oils, sulfurized fatty oils, extreme pressure lubricating agents, organo-metallic compounds, bright stocks (such as refined petroleum lubricating oil residues), volatilized fats, mineral oils and/or waxes, colloidal solids such as graphite, zinc oxide, etc., and the like.

The following examples illustrate the use of these compounds in the preparation of improved lubricating compositions.

#### EXAMPLE VII

A naphthenic petroleum lubricating oil having a viscosity of 55 seconds Saybolt at 210° F. was blended with 1.0% of the thioether of tertiary amyl calcium phenolate (prepared as described in Example II above). Diesel oil oxidation tests on the original oil and the blend gave the following results:

| Oil                     | Diesel oil oxidation tests |         |         |
|-------------------------|----------------------------|---------|---------|
|                         | 48 hrs.                    | 72 hrs. | 96 hrs. |
| Blank oil               | 1                          | 2       | 4       |
| Blank oil +1% inhibitor | 1                          | 1       | 1       |

#### Diesel oil oxidation test

The oil is oxidized at 300° F. for the number of hours indicated. A 10 gram sample is removed and filtered through paper. The deposit

left on the paper is rated from 1 to 10; 1 representing a minimum of deposit and 10 a maximum.

EXAMPLE VIII

Blends of the same oil used in the preceding example with 0.5% of the thioether of tertiary amyl calcium phenolate and of the thioether of tertiary amyl aluminum phenolate were compared as to sludging tendencies with the original oil. The results are given in the following table:

| Oil                            | Sludge test<br>mgs. of<br>sludge |
|--------------------------------|----------------------------------|
| Blank oil                      | 61                               |
| Blank oil + calcium inhibitor  | 32.7                             |
| Blank oil + aluminum inhibitor | 21.9                             |

Sludge test

This test of the tendency of an oil to sludge under oxidizing conditions is described in Proc. A. S. T. M. 24, 964, II (1924), except that the oxidation was conducted for 24 hours.

EXAMPLE IX

Blends of various metal salts of tertiary amyl phenol thioethers prepared by the methods described above in 0.25% concentration in a refined paraffinic petroleum lubricating oil having a viscosity of 77 seconds Saybolt at 210° F. were compared with the original oil by using the oil and the blends thereof as the crankcase lubricant in runs made under closely comparable conditions in a C. F. R. (Cooperative Fuel Research) engine. After each run the engine was taken down, inspected, and rated by demerits according to the condition of the piston parts, valves, and cylinder. On the scale used, the demerit rating of the blank oil is taken as 100. The reference rating for the blends is expressed as a ratio:

$$\frac{\text{Blend demerits}}{\text{Blank oil demerits}} \times 100$$

On this scale the numerical rating is lower as the engine condition is better. The runs were each made for 14 hours at a jacket temperature of 375° F. The results are given in the following table:

| Oil                       | C. F. R.<br>test percent<br>of reference |
|---------------------------|------------------------------------------|
| Blank oil                 | 100                                      |
| Blank oil + aluminum salt | 24                                       |
| Blank oil + barium salt   | 10                                       |
| Blank oil + calcium salt  | 17                                       |
| Blank oil + nickel salt   | 12                                       |
| Blank oil + cobalt salt   | 9                                        |

This invention is not to be limited to any specific examples presented herein, all of such being intended solely for purpose of illustration, but is limited only by the following claims in which it is desired to claim all novelty insofar as the prior art permits.

I claim:

1. Improved lubricant comprising a hydrocarbon lubricating oil and a small proportion of a compound having the formula



in which the groups R, OM, and Z<sub>x</sub>R' are all connected to the aromatic nucleus, and M represents

a metal, R and R' represent organic groups or H, Z represents a member of the sulfur family, and x represents an integer, 1 to 5.

2. Improved lubricant comprising a hydrocarbon lubricating oil and a small proportion of a compound having the formula



in which the groups R, OM, and S are all connected to the aromatic nucleus, and M represents a metal, R and R' represent alkyl groups of 4 to 6 carbon atoms each, and x represents an integer, 1 to 5.

3. Improved lubricating oil composition comprising a hydrocarbon lubricating oil and a small proportion of a sulfide of a metal phenolate.

4. A composition as in claim 3 wherein the metal is calcium.

5. A composition as in claim 3 wherein the metal is tin.

6. A lubricating oil composition comprising a major amount of a hydrocarbon lubricating oil and a minor amount of the calcium salt of an alkyl phenol sulfide in which the alkyl groups each contain between four and eight carbon atoms.

7. A lubricating oil composition comprising a major amount of a hydrocarbon lubricating oil and a minor amount of the calcium salt of a tertiary amyl phenol sulfide.

8. Improved lubricating oil composition comprising a hydrocarbon lubricating oil and a small proportion of a thioether of a metal phenolate.

9. Improved lubricating oil composition comprising a hydrocarbon lubricating oil and a small proportion of a disulfide of a metal phenolate.

10. Improved lubricating oil composition comprising a hydrocarbon lubricating oil and a small proportion of a sulfide of a metal phenolate containing an alkyl group connected to the aromatic nucleus.

11. Composition according to the preceding claim in which the said alkyl group has from 4 to 8 carbon atoms.

12. Improved lubricating oil composition comprising a hydrocarbon lubricating oil and a small proportion of a metal salt of amyl phenol thioether.

13. Improved lubricating oil composition comprising a hydrocarbon lubricating oil and a small proportion of a metal salt of amyl phenol disulfide.

14. A lubricant comprising a major proportion of a mineral lubricating oil having dissolved therein a small amount of a sulfide of a metal salt of an alkylated aryl compound having a hydroxy group attached directly to the aromatic nucleus.

15. A lubricant according to claim 14 in which the sulfide of the metal salt is an oil-soluble metal salt of the reaction product of a sulfur halide with an alkylated aryl compound having a hydroxy group attached directly to the aromatic nucleus.

16. A composition comprising an organic substance which tends to deteriorate by absorption of oxygen from the air and a small proportion of a compound having the general formula R(OM)ArZ<sub>x</sub>R', in which Ar is an aromatic nucleus and in which the groups R, OM, and Z<sub>x</sub>R' are all connected to the aromatic nucleus, and M represents a metal, R and R' represent organic

groups or H, Z represents a member of the sulfur family, and  $x$  represents an integer 1 to 5.

17. A lubricating oil composition comprising a major proportion of a hydrocarbon lubricating oil and a small proportion of a compound having the general formula  $R(OM)ArZ_xR'$ , in which Ar is an aromatic nucleus and in which the groups R, OM, and  $Z_xR'$  are all connected to the aromatic nucleus, and M represents a metal, R and R' represent organic groups or H, Z represents a member of the sulfur family, and  $x$  represents an integer 1 to 5.

18. Improved lubricating oil composition comprising a paraffinic petroleum lubricating oil having dissolved therein a small proportion of a soluble sulfide of a metal phenoate having an alkyl group connected to the aromatic nucleus.

19. Composition according to claim 15 in which the said alkyl group has from four to eight carbon atoms.

20. Composition according to claim 14 in which the said metal is calcium.

21. An improved mineral oil composition comprising a mineral oil having admixed therewith a minor proportion of an oil miscible sulfide of an alkyl substituted aryl metal oxide in which the oxygen of the metal oxide group is directly attached to the aryl nucleus and in which at

least two alkyl substituted aryl nuclei are interconnected by at least one atom of sulfur.

22. Improved lubricant comprising a hydrocarbon lubricating oil and a small proportion of a compound having the formula



10 in which the groups R, OM and  $S_xR'$  are all connected to the aromatic nucleus, and M represents a metal, R and R' represent organic groups and  $x$  represents an integer equal to at least 1.

15 23. A lubricating oil composition comprising a major amount of a hydrocarbon lubricating oil and a minor amount of the metal salt of an oil-soluble aliphatic substituted phenol sulfide, each aliphatic radical containing at least four aliphatic carbon atoms.

20 24. An improved mineral lubricating oil composition comprising a mineral lubricating oil having admixed therewith a minor proportion of an oil-miscible polyvalent metal salt of an alkyl phenol sulfide in which a plurality of phenol groups are attached to a single metal atom.

LOUIS A. MIKESKA.